# EUROPEAN PATENT SPECIFICATION

(11) **EP 3 274 494 B1**
(45) Date of publication and mention of the grant of the patent: **22.12.2021**
(21) Application number: 16718050.4
(22) Date of filing: 24.03.2016
(51) Int. Cl.: D04H 1/435, A41D 31/00, A41G 11/00, B68G 1/00, D04H 1/4391

(54) **BLOWABLE NATURAL DOWN ALTERNATIVE**
BLASBARE NATÜRLICH DAUNENALTERNATIVE
ALTERNATIVE AU DUVET NATUREL GONFLABLE

(30) Priority: 25.03.2015 US 201562138141 P
(43) Date of publication of application: 31.01.2018
(73) Proprietor: 3M Innovative Properties Company, Saint Paul, Minnesota 55133-3427 (US)
(72) Inventor: ROSSBACH, Rebeccah K., Saint Paul, Minnesota 55133-3427 (US); TUMAN, Scott J., Saint Paul, Minnesota 55133-3427 (US); BERRIGAN, Michael R., Saint Paul, Minnesota 55133-3427 (US); NELSON, Brian L., Saint Paul, Minnesota 55133-3427 (US); COX, Kenneth A., Saint Paul, Minnesota 55133-3427 (US)
(74) Representative: Vossius & Partner Patentanwälte Rechtsanwälte mbB
(86) International application number: PCT/US2016/023956
(87) International publication number: WO 2016/154402

(56) References cited:
- EP-A1- 1 717 192
- WO-A2-80/01031
- US-A- 4 618 531
- US-A- 4 992 327
- US-A1- 2014 206 796

## Description

### Background

The present disclosure relates to natural down-like insulation fill materials. More particularly, it relates to a blowable synthetic material comparable to natural down in various performance attributes, methods for manufacturing the same, and articles incorporating the synthetic material as an insulation filler.

A wide variety of natural and synthetic filling material for thermal insulation applications, apparel such as outerwear and accessories (e.g., jackets, stocking caps, gloves, etc.), sleeping bags, and bedding articles (e.g., comforters, pillows, quilts, bedspreads, etc.) are known. Natural feather down has found wide acceptance for thermal insulation applications, primarily because of its outstanding thermal weight efficiency, softness, and resiliency. Properly fluffed and contained within an article or garment, natural down is generally recognized as an insulation material of choice. However, natural down compacts and loses its insulating properties when it becomes wet and can exude a rather unpleasant odor when exposed to moisture. Moreover, the cost of natural down has increased dramatically over the past several years.

To address the above concerns, numerous attempts have been made to prepare synthetic fiber-based structures or materials having the characteristics and structure of natural down. Natural down is very difficult to replicate due to its unique structure and properties; namely, warmth per weight, compressibility, and compression recovery. Further, natural down is readily handled or distributed by the conventional blowing equipment (e.g., a machine or apparatus configured to transport loose fill material via an airstream) utilized by many garment and bedding manufacturers. Unfortunately, prior efforts to develop a feasible replacement material have not met one or more of these desired qualities of natural down. For example, some synthetic fiber-based insulation materials (e.g., the materials described in U.S. Patent Nos. 4,588,635 and 4,992,327) may exhibit warmth per weight properties akin to natural down, but are not easily incorporated as a replacement to down and are not blowable (i.e., cannot be acceptably handled or transported by conventional blowing equipment). Conversely, other synthetic-based insulation materials appropriate for garments and the like purport to be blowable, but do not necessarily compare to natural down in terms of at least warmth and/or compression recovery (e.g., the materials described in U.S. Patent Nos. 6,329,052 and 7,682,693).

In light of the above, a need exists for a blowable synthetic insulation material comparable to natural down in terms of warmth and/or compression/recovery.

### Summary

Some aspects of the present disclosure are directed toward a blend of polyester staple fibers and corresponding insulation fill materials useful as a replacement for natural down in various articles such as outdoor apparel (jackets, hats, gloves, etc.), sleeping bags, and bedding (comforters, pillows, etc.). The polyester staple fiber blend includes a plurality of first polyester staple fibers, a plurality of second polyester staple fibers, and a plurality of third polyester staple fibers. An average Denier of each of the second polyester staple fibers is greater than an average Denier of each of the first polyester staple fibers. An average Denier of each of the third polyester staple fibers is greater than an average Denier of each of the second polyester staple fibers. Further, a length of substantially all the fibers of the blend is in the range of 16 - 63 mm, alternatively in the range of 20 - 40 mm. Additionally, at least a majority, optionally substantially all, of the fibers of the blend are opened. In some embodiments, some or substantially all of the fibers of the blend are crimped; in other embodiments, some or substantially all of the fibers of the blend include a lubricant (e.g., are siliconized). In one non-limiting embodiment, the blend of polyester staple fibers includes 20 - 30 weight percent of not greater than about 1 Denier polyester staple fibers, 20 - 30 weight percent of greater than about 1 up to about 2 Denier polyester staple fibers, and 40 - 60 weight percent of greater than about 2 Denier polyester staple fibers, with substantially all of the fibers of the blend each having a length in the range of 20 - 40 mm. The polyester staple fiber blends of the present disclosure are blowable and may exhibit superior performance in terms of warmth, compression/recovery, and wash durability.

### Brief Description of the Drawings

FIG. 1 is a simplified cross-sectional view of an article including a polyester staple fiber blend in accordance with principles of the present disclosure;
FIG. 2 is a schematic illustration of a system for manufacturing the polyester staple fiber blends in accordance with principles of the present disclosure; and
FIG. 3 and 4 are graphs illustrating the results of Warmth/Heat Transfer Resistance testing described in the Examples section.

### Detailed Description

Aspects of the present disclosure provide an insulation material comprised of a blend or mixture of polyester staple fibers. The blend includes three different polyester staple fiber formats or types. Further, the blend is blowable (e.g., the fibers of the blend are collectively loose filled or opened) and exhibits warmth or heat transfer resistance characteristics comparable to natural down. In some embodiments, the blowable insulation material of the present disclosure is comprised essentially of the blend of polyester staple fibers, and may exhibit superior performance in terms of warmth (e.g., warmth per thickness (or thermal resistivity), and/or warmth per basis weight (or thermal weight efficiency)), compression/recovery, and/or wash durability.

The fibers of the polyester staple fiber blends of the present disclosure are selected from one of three polyester staple fiber formats or types. For ease of explanation, the fiber formats or types are referred to as Fiber Format A, Fiber Format B, and Fiber Format C. While the fibers of the three Fiber Formats can have similarities (e.g., base polymer composition and length), Fiber Format A, Fiber Format B, and Fiber Format C differ from one another at least in terms of average Denier as described in greater detail below.

For example, all of the polyester staple fibers of the blend (and thus the fibers of each of the Fiber Formats A, B and C) can be single component in nature, formed from a similar or identical polyester material such as, but not limited to: polyethylene terephthalate (PET). In some embodiments, the fibers of each of the three Fiber Formats are PET. In other embodiments, the fibers of one of the Fiber Format can have a polyester formulation differing from the polyester formulation of the other Fiber Formats. In other embodiments, the fibers may include other synthetic fibers, including, but not limited to, polymers or combinations of: polyesters, polyamides, polyolefins, polyacrylates, and polyaramids.

Further, substantially all (e.g., at least 95%, optionally at least 98%, optionally at least 99%) of the polyester staple fibers of the blend (and thus the fibers of Fiber Formats A, B and C) are cut to a length in the range of 16 - 63 mm, optionally in the range of 20 - 40 mm, optionally on the order of 32 mm. It has been surprisingly found that the fiber lengths of the present disclosure beneficially render the blend of polyester stable fibers, and thus the insulation materials of the present disclosure, conducive to handling or distribution by conventional blowing equipment.

An additional, optional similarity of the fibers comprising the polyester staple fiber blend (and thus the fibers of Fiber Formats A, B and C) relates to crimping. For example, a majority, optionally substantially all (e.g., at least 95%, optionally at least 98%, optionally at least 99%), of the polyester staple fibers of the blend (and thus a majority or substantially all of the fibers of Fiber Formats A, B or C comprising the blend) are crimped (e.g., two-dimensional mechanical crimp, spiral crimp, etc.), for example having 1 - 10 crimps/cm. In other embodiments, substantially all of the fibers of at least one of the Fiber Formats comprising the polyester staple fiber blend are crimped fibers, whereas a majority or substantially all of the fibers of another Fiber Format comprising the polyester staple fiber blend are not crimped. In yet other embodiments, substantially all of the fibers of the polyester staple fiber blend are not crimped.

An additional, optional similarity of the fibers comprising the polyester staple fiber blend (and thus the fibers of Fiber Formats A, B and C) relates to lubricants, and in particular the addition of a lubricant or slickening agent (e.g., a silicone slickener, aqueous solutions of organopolysiloxanes, emulsions of polytetrafluoroethylene, non-ionic surfactants, etc.) for water resistance, improved feel and/or handling, and antistatic properties. The lubricant can be applied (e.g., spray coated) on to an exterior surface of the polyester staple fibers, or can be added to the polyester material during formation of the corresponding fibers (e.g., at the spinning stage prior to drawing). With this in mind, in some embodiments a majority, optionally substantially all (e.g., at least 95%, optionally at least 98%, optionally at least 99%), of the polyester staple fibers of the blend (and thus a majority, optionally substantially all, of the fibers of Fiber Formats A, B or C comprising the blend) include a lubricant (e.g., are siliconized polyester fibers). In other embodiments, substantially all of the fibers of at least one of the Fiber Formats comprising the polyester staple fiber blend include a lubricant, whereas a majority or substantially all of the fibers of another Fiber Format comprising the polyester staple fiber blend do not include a lubricant. In yet other embodiments, substantially all of the fibers of the polyester staple fiber blend do not include a lubricant.

As mentioned above, while Fiber Formats A, B and C can have certain similarities, the fibers of Fiber Formats A, B and C differ from one another at least in terms of average Denier or cross-dimensional size. In particular, the polyester staple fibers of Fiber Format A have a Denier of not greater than about 1 Denier, optionally a Denier in the range of about 0.5 to not greater than about 1 Denier, optionally on the order of 0.7 Denier. The polyester staple fibers of Fiber Format B have a Denier in the range of greater than about 1 Denier to not greater than about 2 Denier, optionally on the order of 1.4 Denier. The polyester staple fibers of Fiber Format C have a Denier greater than about 2 Denier, optionally in the range of about greater than 2 Denier to 7 Denier, optionally on the order of 3 Denier.

An additional, optional difference between the fibers of at least one of the Fiber Formats relates to structure. In particular, some of the fibers comprising the polyester staple fiber blend can be solid, whereas others of the fibers comprising the polyester staple fiber blend can be hollow or tubular. For example, a majority, optionally substantially all (e.g., at least 95%, optionally at least 98%, optionally at least 99%), of the fibers of a first one of the Fiber Formats comprising the blend (i.e., Fiber Format A, B or C) are solid; whereas a majority, optionally substantially all (e.g., at least 95%, optionally at least 98%, optionally at least 98%), of the fibers of a second one of the Fiber Formats comprising the blend (i.e., Fiber Format A, B or C) are hollow. By way of one non-limiting example, some polyester staple fiber blends in accordance with principles of the present disclosure consist include fibers of Fiber Format A and Fiber Format B is solid form, and fibers of Fiber Format C in hollow form. In other embodiments, substantially all of the fibers of the blend are hollow regardless of Fiber Format; in yet other embodiments, substantially all of the fibers of the blend are solid regardless of Fiber Format. Fibers can be circular or other shapes in cross sections such as triangular.

With the above characteristics of Fiber Formats A, B and C in mind, the polyester staple fiber blends of the present disclosure comprise, optionally consist essentially of, fibers from Fiber Formats A, B, and C. In some embodiments, the polyester staple fiber blends of the present disclosure are comprised of 20-30 weight percent of Fiber Format A, 40 - 60 weight percent of Fiber Format B, and 40 - 60 weight percent of Fiber Format C.

Regardless of an exact composition, the polyester staple fiber blends of the present disclosure can be characterized as loose fill, with at least a majority of the fibers comprising the blend being opened (as commonly understood to those of ordinary skill in the art). That is to say, at least a majority, alternatively at least about 70%, and in other optional embodiments substantially all (e.g. at least 95%, alternatively at least 98%, alternatively at least 99%), of the fibers comprising the blend are separated, individualized and unbonded relative to one another. The "opening" of the fibers of the polyester staple fiber blend means that the fibers are worked upon such that the individual fibers of the blend are separated from each other and are not clustered. Opening of the fibers of the staple fiber blend can be accomplished by various methods known in the art as described in greater detail below.

In some embodiments, the insulation materials of the present disclosure consist substantially, alternatively solely, of the polyester staple fiber blend as described above. In other embodiments, the insulation materials can include one or more components in addition to the polyester staple fiber blend, such as other synthetic fibers, natural fibers, natural down, and fiber clusters. Other possible additives envisioned by the present disclosure include benefitting additives such as chopped sponge, anti-microbials, abrasives, odor absorbing particulate, adhesive/binder particulate (e.g., heat activatable, moisture transporting particulate, heat conducting particulate (e.g., inorganic, metallic, crushed gemstones), radiation blocking (UV/visible/IR), detergent/soap, wetting agents, microencapsulants (phase change materials, fragrance, essential oils, etc.), flame retardants, etc.

The insulation materials described above can be incorporated into various articles. For example, FIG. 1 is a simplified view of a portion of an article 10 in accordance with principles of the present disclosure. The article 10 can assume a variety of forms, such as apparel including outerwear and accessories (e.g., jackets, stocking caps, gloves, etc.), sleeping bag, bedding articles (comforters, pillows, quilts, bedspreads, etc.), and generally includes a quantity or volume of the blend of polyester staple fibers 12 as described above contained within a pocket 14 formed by an outer shell or liner 16 (e.g., fabric, film, etc.). In some embodiments, construction of the article 10 includes dispensing or filling the blend of polyester staple fibers 12 into the pocket 14 with a conventional blowing device (i.e., the blend of polyester staple fibers 12 is delivered into the pocket 14 via a forced airstream).

Various methods can be employed in accordance with principles of the present disclosure to manufacture the polyester staple fiber blends described above. In general terms, desired quantities of fibers of Fiber Format A, Fiber Format B and Fiber Format C, in accordance with the weight percent selected for the resultant blend, are obtained. The polyester fibers can be obtained, for instance, by conventional spinning/drawings or extrusion techniques as known in the art, and can be cut to the lengths described above. The so-obtained fibers may be crimped and may include a lubricant as described above. Regardless, the fibers are then mixed and opened to produce the polyester staple fiber blend of the present disclosure and useful as a blowable insulation material.

One non-limiting example of a system 20 (and corresponding method) for producing the polyester stable fiber blends of the present disclosure is provided in FIG. 2. Raw polyester staple fibers are received at a loading station 22. The loading station 22 can include three (or more) pre-feeder substations 22a-22c each including a weighing pan (as known in the art), one for each of the Fiber Formats to be included with the resultant blend. For example, FIG. 2 reflects fibers of Fiber Format A being loaded on to the first pre-feeder substation 22a, fibers of Fiber Format B being loaded on to the second pre-feeder substation 22b, and fibers of Fiber Format C being loaded on to the third pre-feeder substation 22c. The raw polyester staple fibers can be supplied in bale form, can be formed substantially in-line with the system 20, etc. Once a desired quantity of the each of the Fiber Formats A, B and C has been obtained (e.g., based on weight), the quantities are dispensed from the corresponding pre-feeder substation 22a-22c on to a conveyor 24. The conveyor 24 operates to deliver the quantities of fiber to a mixing station 26. The mixing station 26 can assume include various mechanisms appropriate for effectuating mixing of the fibers as known in the art, such as a turbulent airstream. The mixing station 26 can further operated to effectuate coarse opening of the fibers.

The mixed blend of polyester staple fibers (identified generally at 28 in FIG. 2) is then fed to a fine opening station 30 configured to effectuate more complete or full opening of substantially all of the fibers of the blend. The fine opening station 30 can assume various forms and can incorporate various mechanisms for "working" or opening the fibers, such as rotating or vibrating pins or shafts, compressed air, etc. The systems and methods of the present disclosure can further include additional opening stations downstream of the fine opening station 30 and that utilize other fiber opening techniques. In other embodiments, the mixing station 26 alone interfaces with the fibers to sufficiently generate desired openness.

The blend of opened polyester staple fibers (referenced generally at 32 in FIG. 2) is then fed to one or more gathering stations 34. The gathering station(s) 34 can assume various forms, and in some embodiments each include a chute 36 (or other feeding apparatus) and a carding machine 38 (e.g., a Double Doffer carder). The so-gathered blend of polyester staple fibers is then prepared for delivery to an end user/manufacturer (e.g., packaged or bagged) for use as a blowable insulation fill material.

### EXAMPLES AND COMPARATIVE EXAMPLES

Objects and advantages of the present disclosure are further illustrated by the following non-limiting examples and comparative examples. The particular materials and amounts thereof recited in these examples, as well as other conditions and details, should not be construed to unduly limit the present disclosure.

Unless otherwise noted, all parts, percentages, ratios, etc. in the Examples and the rest of this specification are by weight.

A first example of a polyester staple fibers blend ("Example Blend A") in accordance with principles of the present disclosure was prepared and consisted of: 1) 30 weight percent of crimped, siliconized, solid polyester staple fibers of 0.7 Denier and an average length of 32 mm (e.g., Fiber Format A); 2) 30 weight percent of crimped, solid polyester staple fibers of 1.4 Denier and an average length of 38 mm (e.g., Fiber Format B); 3) 40 weight percent of crimped, siliconized, hollow polyester staple fibers of 3 Denier and an average length of 32 mm (e.g., Fiber Format C).

A second example of a polyester staple fibers blend ("Example Blend B") in accordance with principles of the present disclosure was prepared and consisted of: 1) 60 weight percent of crimped, siliconized, solid polyester staple fibers of 0.7 Denier and an average length of 32 mm (e.g., Fiber Format A); 2) 20 weight percent of crimped, siliconized, hollow polyester staple fibers of 3 Denier and an average length of 32 mm (e.g., Fiber Format B); 3) 20 weight percent of crimped, siliconized, hollow polyester staple fibers of 7 Denier and an average length of 32 mm (e.g., Fiber Format C).

### Blowability Testing

Blowability (or loose fill properties) was tested by evaluating handling of the material by a conventional blowing machine, and in particular a natural down filling or blowing machine available from B&B di Borsio of Tarzo, Italy under the trade designation "Alan PE". The Alan PE blowing machine includes an inlet or feeding chamber and an outlet or injector reducer. Further, the Alan PE blowing machine provides for variable speeds of operation, and includes a variable speed controller dial with eleven speed setting ("0" being the lowest speed setting, and "10" being the highest). Handful-sized samples (approximately 13 grams of material was divided into 10 handful size samples (1-2 grams each sample)) of Example Blend A were prepared. A first one of the samples was placed in the feeding chamber, and the variable speed controller was set to the highest velocity ("10"). The blowing machine was then activated and a manual determination made as to whether or not the sample passed through the machine (e.g., exited the injector reducer) without plugging (e.g., signs of reduced air output, ability to see light through the injector reducer, etc.). If it was determined that the sample passed through without plugging, Example Blend A was designated has having been successfully blown at the particular speed setting; the variable speed controller setting was then reduced by 1 increment, and the steps repeated with a new the samples. If it was determined that plugging occurred, the blowing machine was first cleared of the blockage, and the process repeated three additional times ("trials") at the same speed setting. If all three trials did not result in plugging, Example Blend A was designated as being blowable (i.e., successfully blown) at the particular speed setting; the variable speed controller setting was then reduced by 1 increment, and the steps repeated with a new sample. If two consecutive instances of plugging at a particular speed setting were detected, Example Blend A was designated as not blowable (i.e., unsuccessfully blown) at the particular speed setting or at any lower speed settings, and the testing discontinued.

For purposes of comparison, the above-described blowability test was performed using samples of natural down (Comparative Example 1) and using samples of an openedsynthetic fiber material consisting of 3 Denier x 64 mm crimped, siliconized, hollow polyester staple fibers (Comparative Example 2). Results of the blowability testing are reported in Table 1, where "S" represents that the sample in question was designated to be successfully blown (i.e., no plugging) at the corresponding velocity setting, and "U" represents that the sample in question was designated to not be successfully blown at the corresponding velocity setting.

**Table 1 - Blowability**

| | Velocity Setting | | | | | | | | | | |
|---|---|---|---|---|---|---|---|---|---|---|---|
| Sample | 10 | 9 | 8 | 7 | 6 | 5 | 4 | 3 | 2 | 1 | 0 |
| Comp Ex 1 | S | S | S | S | S | S | S | S | S | S | S |
| Comp Ex 2 | S | S | S | S | S | S | U | U | U | U | U |
| Example Blend A | S | S | S | S | S | S | S | S | U | U | U |

As reflected by the test results, Example Blend A is blowable with conventional blowing equipment, and is more readily handled in a moving airstream than 3 Denier x 64 mm polyester staple fibers (that are otherwise considered highly useful as garment insulation material filler).

### Warmth/Heat Transfer Resistance Testing

Warmth (heat transfer resistance, in units of Clo) of Example Blend A was measured in accordance with ASTM C518-10 (2010) as described below. The warmth properties of comparative example insulation filling materials were similarly tested. The Comparative Examples included:
Comparative Example 3. A jacket available from Nike, Inc. under the trade designation "SB 700 Down" was obtained, and the down fill material was harvested from the jacket's shell and prepared into a standard construction for assessment. The down fill material of Comparative Example 3 is advertised as a 700 fill power down.
Comparative Example 4. A jacket available from Columbia Sportswear Co under the trade designation "Men's Upper Slopes II Down Jacket" was obtained, and the down filler material was harvested from the jacket's shell and prepared into a standard construction for assessment. The down filler material of Comparative Example 4 is advertised as a 700 fill power down.
Comparative Example 5. A jacket available from The North Face (a division of VF Outdoor, Inc.) under the trade designation "Men's Nuptse Jacket" was obtained, and the down fill material was harvested from the jacket's shell and prepared into a standard construction for assessment. The down fill material of Comparative Example 5 is advertised as a 700 fill power down.
Comparative Example 6. A jacket available from The North Face (a division of VF Outdoor, Inc.) under the trade designation "Men's Iron Jacket" was obtained, and the down fill material was harvested from the jacket's shell and prepared into a standard construction for assessment. The down fill material of Comparative Example 6 is advertised as a 700 fill power down.
Comparative Example 7. A down alternative, synthetic fiber insulation fill material available from The North Face (a division of VF Outdoor, Inc.; developed in partnership with PrimaLoft, Inc.) under the trade designation "ThermoBall Powered by PrimaLoft". The fill material of Comparative Example 7 is advertised as being equivalent to 600 fill power down.
Comparative Example 8. A down alternative, synthetic fiber insulation fill material available from PrimaLoft, Inc. under the trade designation "PrimaLoft Luxe".
Comparative Example 9. An insulation fill material comprising a 60-40 blend of down and synthetic fibers available from PrimaLoft, Inc. under the trade designation "PrimaLoft Silver Down Blend". The fill material of Comparative Example 9 is advertised as being equivalent to 650 fill power down.
Comparative Example 10. A natural down alternative, synthetic fiber insulation fill material available from 3M Company under the trade designation "3M Thinsulate Featherless Insulation - 600" was obtained and prepared into a standard construction for assessment. The fill material of Comparative Example 10 is advertised as mimicking600 fill power down.
Comparative Example 11. An insulation fill material comprising a 70-30 blend of down and synthetic fibers available from PrimaLoft, Inc. under the trade designation "PrimaLoft Gold Down Blend". The fill material of Comparative Example 11 is advertised as being equivalent to 750 fill power down.

Test specimens were prepared by quilting 200 gsm (grams per meter² ) loose material samples of Example Blend A and Comparative Examples 3-11 into approximately 12 inch x 12 inch (30.5 cm x 30.5 cm) panels with approximately 3 inch (7.6 cm) pleat spacing. First, 12 inch x 12 inch (30.5 cm x 30.5 cm) fabric sheets were obtained from a 104 x 104 thread count 1.9 oz/yd² (64.4 gsm) Nylon Ripstop (5 ribs per inch (2.54 cm)) fabric. Two of the fabric sheets were aligned and then sewn to one another along three of the four common edges to provide a panel forming a pocket which was then inverted prior to filling. Comparative Example test specimens using the samples of Comparative Examples 3-11 were prepared by evenly distributing the 200 gsm sample into the pocket, followed by sewing quilt lines across the panel at 3 inch (7.6 cm) increments. A first Example test specimen using a 200 gsm sample of Example Blend A was prepared in an identical manner ("Example A-1"). A second Example test specimen using a 200 gsm sample of Example Blend A was prepared by a "channel fill" method in which pre-sewing quilt lines were first formed across the panel at 3 inch (7.6 cm) increments to define four channels; the Example Blend 1 sample (200 gsm) was then filled into each of the so-formed channels ("Example A-2"). All of the test specimens were conditioned for 24 hours in a CTH room set to 21 ± 2°C and 50 ± 2% RH. In some instances if the fiber blend materials had become compressed due to handling (i.e., storage or shipping) the fibers were re-lofted by hand carding.

The thickness of each of the test specimens was recorded, and heat transfer resistance (warmth) was calculated in accordance with ASTM C518-10 (2010). The so-obtained heat transfer resistance value for each test specimen was calculated (in units of Clo). The results of the warmth testing are reported in the graphs of FIGS. 3 and 4. FIG. 3 provides a comparison of the recorded thickness and warmth values of Comparative Example 3-6 test specimens, Example Blend A-1 test specimen, and Example Blend A-2 test specimen. FIG. 4 provides a comparison of the recorded thickness and warmth values of Comparative Examples 7-11 test specimens and Example Blend A-1 test specimen.

The warmth testing results indicate that Example Blend A is comparable to that of typical 700 fill power down (FIG. 3). It was observed that the method of construction (direct sew (Example Blend A-1 test specimen) vs. channel fill (Example Blend A-2 test specimen)) may more substantively impact the thickness of the test panel and subsequent heat transfer resistance (Clo) results with Example Blend A as compared to the natural down Comparative Examples. In addition, the warmth testing results indicate that warmth performance of Example Blend A exceeds that of several existing synthetic fiber insulation fill materials and is comparable to that of existing natural down-synthetic fiber blend insulation fill materials (FIG. 4). Example Blend A was observed as having beneficial warmth per thickness (or thermal resistivity) characteristics.

### Compression-Recovery Testing

Compression-Recovery properties were measured in accordance with ASTM D6571-01 (2001) except as listed below. Test specimens were prepared pursuant to the descriptions of the Warmth/Heat Transfer Resistance Testing section above with the "channel fill" method, using samples of Example Blend A, Example Blend B, and Comparative Example 6 (natural down).

Compression-Recovery testing of the respective Examples and Comparative Examples began by stacking several of the corresponding test specimens between the plates of a loading device commensurate with that of ASTM D6571-01 (2001). A number of masses were then centrally and uniformly placed on the specimen stack to get the correct total mass in accordance with that of ASTM D6571-01 (2001). The initial height of the so-prepared specimen stack was measured and recorded (A). After a 24-hour test period, the height of the compressed specimen stack was measured and recorded (G). Percent Compression was determined as: 100 (A-G)/A. The mass was removed and the specimen stack was allowed to relax for one hour. After the one hour recovery period, the height of the specimen stack was measured and recorded, and Percent Short Term Recovery was determined as: 100 J/E.

The results of the Compression-Recovery Testing are reported in Table 2.

**Table 2 - Compression/Recovery**

| Sample | Initial Height (cm) | Height after 24 hours (cm) | Height Change (cm) | % Compression | % Short Term Compression Recovery |
|---|---|---|---|---|---|
| Example Blend A | 9.8 | 1.3 | 8.6 | 87 | 80 |
| Example Blend B | 9.6 | 1.2 | 8.4 | 87 | 79 |
| Comp Ex 6 | 8.5 | 1.6 | 6.9 | 81 | 77 |

### Wash Durability Testing

Wash durability was evaluated by subjecting test specimens (described below) to the following testing. Prior to washing in a conventional automatic washing machine, a thickness and warmth value (in units of Clo as tested and calculated by ASTM C518-10 (2010)) of the test specimen was measured and recorded. The washing machine settings were selected as "super load fill level", a cold water wash, cold water rinse, delicate cycle, and regular soil wash setting. 16 grams of powdered laundry detergent (TIDE. Procter & Gamble Co.) was added to the washing machine's tub, and the washing cycle initiated. After allowing the tub to fill with water for 20-30 seconds, 3-6 test specimens were added to the washing machine's tub along with three ballast items (pre-washed and cleaned fabric bath towels). When the wash cycle was complete, the entire load was transferred to a conventional automatic clothes dryer. The dryer was set to "delicate". Three clean tennis balls (pre-washed before use) were then added to the dryer. After 60 minutes drying time, the test specimen was removed. Thickness and warmth value of the washed/dried test specimen was measured and recorded after 24 hours of conditioning in the CTH room set to 21 ± 2°C and 50 ± 2% RH An exterior of the washed/dried test specimen was visually evaluated along at least one channel of the specimen and rated on a scale of 1-5 according to the guidelines of Table 3. Further, the washed/dried test specimen was cut open and an interior of at least one channel of the test specimen was visually evaluated on a scale of 1-5 according to the guidelines of Table 3.

**Table 3 - Rating System**

| Rating | Description |
|---|---|
| 1 | Channel has large areas with no material, and feels stiff or hard to the touch, little or no loft |
| 2 | Channel has multiple small areas with little or no material, and feels less stiff with potential balling or pilling of the material, has some loft |
| 3 | Channel has few areas missing material with some areas that might be low on material, feels moderately soft with minor balling or piling, has good loft |
| 4 | Channel has few areas with low or missing material, feels soft with minor balling, has good loft |
| 5 | Channel has no areas with low or missing material, feels extremely soft with no noticeable balling, has natural down-like loft |

Test specimens for Wash Durability Testing were prepared pursuant to the descriptions of the Warmth/Heat Transfer Resistance Testing section above, using samples of Example Blend A and Comparative Example 8. The results of the Wash Durability Testing are reported in Table 4.

**Table 4 - Wash Durability Testing**

| Sample | Thickness (cm) | Warmth (Clo) | Rating - External | Rating - Internal |
|---|---|---|---|---|
| Example Blend A before wash/dry | 4.42 | 5.36 | - | - |
| Example Blend A after wash/dry | 3.52 | 4.49 | 5 | 5 |
| Comp Ex 8 before wash/dry | 4.14 | 5.02 | - | - |
| Comp Ex 8 after wash/dry | 2.50 | 3.58 | 4 | 4 |

The blowable insulation materials and corresponding blend of polyester staple fibers of the present disclosure provide an improvement over previous designs. The polyester staple fiber blends of the present disclosure are readily transported by the airstream of conventional blowing equipment utilized to fill garments and the like with natural down. Further, the polyester staple fiber blends of the present disclosure are highly comparable to typical 700 fill power down in terms of warmth and compression/recovery, including beneficial warmth per thickness (thermal resistivity) properties. Moreover, the polyester staple fiber blends of the present disclosure exhibit better performance as compared to some existing down alternative products in terms of wash durability and are hypoallergenic.

Although the present disclosure has been described with reference to preferred embodiments, workers skilled in the art will recognize that changes can be made in form and detail without departing from the scope of the present disclosure.

## Claims

1. A blowable insulation material comprising:
a blend of polyester staple fibers including a plurality of first polyester staple fibers, a plurality of second polyester staple fibers, and a plurality of third polyester staple fibers;
wherein a Denier of each of the second polyester staple fibers is greater than a Denier of each of the first polyester staple fibers;
wherein a Denier of each of the third polyester staple fibers is greater than a Denier of each of the second polyester staple fibers;
wherein each of the first polyester staple fibers has a Denier of not greater than about 1 Denier, each of the second polyester staple fibers has a Denier in the range of not less than about 1 Denier to not greater than about 2 Denier, and each of the third polyester staple fibers has a Denier of not less than about 2 Denier;
wherein a length of substantially all of the polyester staple fibers of the blend is in the range of about 16 to about 63 mm;
wherein the fibers of at least one of the first and second polyester staple fibers are polyethylene terephthalate;
wherein at least a majority of the polyester staple fibers of the blend are opened; and
wherein the fibers comprising the blend are separated, individualized and unbonded relative to one another.

2. The blowable insulation material of claim 1, wherein the blend comprises about 20 to about 40 weight percent of the first polyester staple fibers, about 20 to about 30 weight percent of the second polyester staple fibers, and about 40 to about 60 weight percent of the third polyester staple fibers.

3. The blowable insulation material of claim 1, wherein the length of each of the polyester staple fibers of the blend is in the range of about 20 to about 30 mm.

4. The blowable insulation material of claim 1, wherein at least about 95% of the polyester staple fibers of the blend are opened.

5. The blowable insulation material of claim 1, wherein the fibers of at least one of the first polyester staple fibers and the second polyester staple fibers includes a lubricant.

6. The blowable insulation material of claim 5, wherein the lubricant 5 is silicone.

7. The blowable insulation material of claim 1, wherein the fibers of at least one of the first polyester staple fibers and the second polyester staple fibers are crimped.

8. The blowable insulation material of claim 1, wherein the blend exhibits a heat transfer resistance of 700 fill power down.

9. An article comprising an outer shell containing a volume of the blowable insulation material of claim 1.

10. A supply of insulation material for filling at least a segment of a shell of a garment via a blowing apparatus, the insulation material comprising:
a blend of polyester staple fibers including a plurality of first polyester staple fibers, a plurality of second polyester staple fibers, and a plurality of third polyester staple fibers;
wherein a Denier of each of the second polyester staple fibers is greater than a Denier of each of the first polyester staple fibers;
wherein a Denier of each of the third polyester staple fibers is greater than a Denier of each of the second polyester staple fibers;
wherein each of the first polyester staple fibers has a Denier of not greater than about 1 Denier, each of the second polyester staple fibers has a Denier in the range of not less than about 1 Denier to not greater than about 2 Denier, and each of the third polyester staple fibers has a Denier of not less than about 2 Denier;
wherein a length of each of the polyester staple fibers of the blend is in the range of about 16 to about 63 mm;
wherein at least a majority of the polyester staple fibers of the blend are opened; and
wherein the fibers comprising the blend are separated, individualized and unbonded relative to one another.

11. A method for preparing a supply of blowable insulation material, the method comprising:
obtaining a quantity of first polyester staple fibers;
obtaining a quantity of second polyester staple fibers;
obtaining a quantity of third polyester staple fibers, wherein an average Denier of each of the second polyester staple fibers is greater than an average Denier of each of the first polyester staple fibers, wherein an average Denier of each of the third polyester staple fibers is greater than an average Denier of each of the second polyester staple fibers,
wherein each of the first polyester staple fibers has a Denier of not greater than about 1 Denier, each of the second polyester staple fibers has a Denier in the range of not less than about 1 Denier to not greater than about 2 Denier, and each of the third polyester staple fibers has a Denier of not less than about 2 Denier, wherein each of the first polyester staple fibers and each of the second polyester staple fibers has a length in the range of about 16 to about 63 mm, and wherein the fibers comprising the blend are separated, individualized and unbonded relative to one another; and
mixing the quantities of first, second, and third polyester staple fibers to provide a blend of polyester staple fibers useful as a supply of blowable insulation material.

## Patentansprüche

1. Ein blasbares Isoliermaterial, aufweisend:
eine Mischung aus Polyesterstapelfasern, die eine Mehrzahl von ersten Polyesterstapelfasern, eine Mehrzahl von zweiten Polyesterstapelfasern und eine Mehrzahl von dritten Polyesterstapelfasern aufweist;
wobei ein Denier von jeder der zweiten Polyesterstapelfasern größer ist als ein Denier von jeder der ersten Polyesterstapelfasern;
wobei ein Denier von jeder der dritten Polyesterstapelfasern größer ist als ein Denier von jeder der zweiten Polyesterstapelfasern;
wobei jede von den ersten Polyesterstapelfasern ein Denier von nicht größer als etwa 1 Denier hat, jede von den zweiten Polyesterstapelfasern ein Denier im Bereich von nicht weniger als etwa 1 Denier bis nicht größer als etwa 2 Denier hat und jede von den dritten Polyesterstapelfasern ein Denier von nicht weniger als etwa 2 Denier hat;
wobei eine Länge von im Wesentlichen allen Polyesterstapelfasern der Mischung im Bereich von etwa 16 bis etwa 63 mm liegt;
wobei die Fasern von mindestens einen von den ersten und zweiten Polyesterstapelfasern Polyethylenterephthalat sind;
wobei mindestens ein Großteil der Polyesterstapelfasern der Mischung geöffnet sind; und wobei die Fasern, die die Mischung umfassen, in Bezug zueinander getrennt, individualisiert und ungebunden sind.

2. Das blasbare Isoliermaterial nach Anspruch 1, wobei die Mischung zu etwa 20 bis etwa 40 Gewichtsprozent die ersten Polyesterstapelfasern, zu etwa 20 bis etwa 30 Gewichtsprozent die zweiten Polyesterstapelfasern und zu etwa 40 bis etwa 60 Gewichtsprozent die dritten Polyesterstapelfasern aufweist.

3. Das blasbare Isoliermaterial nach Anspruch 1, wobei die Länge von jeder der Polyesterstapelfasern der Mischung im Bereich von etwa 20 bis etwa 30 mm liegt.

4. Das blasbare Isoliermaterial nach Anspruch 1, wobei mindestens etwa 95 % der Polyesterstapelfasern der Mischung geöffnet sind.

5. Das blasbare Isoliermaterial nach Anspruch 1, wobei die Fasern von mindestens einer der ersten Polyesterstapelfasern und der zweiten Polyesterstapelfasern ein Gleitmittel enthalten.

6. Das blasbare Isoliermaterial nach Anspruch 5, wobei das Gleitmittel 5 Silikon ist.

7. Das blasbare Isoliermaterial nach Anspruch 1, wobei die Fasern von mindestens einer der ersten Polyesterstapelfasern und der zweiten Polyesterstapelfasern gekräuselt sind.

8. Das blasbare Isoliermaterial nach Anspruch 1, wobei die Mischung einen Wärmeübergangswiderstand von Daunenbauschkraft 700 aufweist.

9. Ein Gegenstand, aufweisend eine Außenhülle, die ein Volumen des blasbaren Isoliermaterials nach Anspruch 1 enthält.

10. Eine Zufuhr von Isoliermaterial zum Füllen mindestens eines Segments einer Hülle eines Kleidungsstücks mittels einer Blasvorrichtung, wobei das Isoliermaterial aufweist:
eine Mischung aus Polyesterstapelfasern, die eine Mehrzahl von ersten Polyesterstapelfasern, eine Mehrzahl von zweiten Polyesterstapelfasern und eine Mehrzahl von dritten Polyesterstapelfasern aufweist;
wobei ein Denier von jeder der zweiten Polyesterstapelfasern größer ist als ein Denier von jeder der ersten Polyesterstapelfasern;
wobei ein Denier von jeder der dritten Polyesterstapelfasern größer ist als ein Denier von jeder der zweiten Polyesterstapelfasern;
wobei jede von den ersten Polyesterstapelfasern ein Denier von nicht größer als etwa 1 Denier hat, jede von den zweiten Polyesterstapelfasern ein Denier im Bereich von nicht weniger als etwa 1 Denier bis nicht größer als etwa 2 Denier hat und jede von den dritten Polyesterstapelfasern ein Denier von nicht weniger als etwa 2 Denier hat;
wobei eine Länge von jeder der Polyesterstapelfasern der Mischung im Bereich von etwa 16 bis etwa 63 mm liegt;
wobei mindestens ein Großteil der Polyesterstapelfasern der Mischung geöffnet sind; und wobei die Fasern, die die Mischung aufweisen, in Bezug zueinander getrennt, individualisiert und ungebunden sind.

11. Ein Verfahren zum Vorbereiten einer Zufuhr an blasbarem Isoliermaterial, wobei das Verfahren aufweist:
Erhalten einer Menge an ersten Polyesterstapelfasern;
Erhalten einer Menge an zweiten Polyesterstapelfasern;
Erhalten einer Menge an dritten Polyesterstapelfasern, wobei ein durchschnittliches Denier von jeder der zweiten Polyesterstapelfasern größer ist als ein durchschnittliches Denier von jeder der ersten Polyesterstapelfasern, wobei ein durchschnittliches Denier von jeder der dritten Polyesterstapelfasern größer ist als ein durchschnittliches Denier von jeder der zweiten Polyesterstapelfasern,
wobei jede von den ersten Polyesterstapelfasern ein Denier von nicht mehr als etwa 1 Denier hat, jede von den zweiten Polyesterstapelfasern ein Denier im Bereich von nicht weniger als etwa 1 Denier bis nicht größer als etwa 2 Denier hat und jede von den dritten Polyesterstapelfasern ein Denier von nicht weniger als etwa 2 Denier hat, wobei jede von den ersten Polyesterstapelfasern und jede von den zweiten Polyesterstapelfasern eine Länge im Bereich von etwa 16 bis etwa 63 mm hat, und wobei die Fasern, die die Mischung aufweisen, in Bezug zueinander getrennt, individualisiert und ungebunden sind; und
Mischen der Mengen von ersten, zweiten und dritten Polyesterstapelfasern, um eine Mischung von Polyesterstapelfasern bereitzustellen, die als eine Zufuhr an blasbarem Isoliermaterial nützlich ist.

## Revendications

1. Matériau d'isolation soufflable comprenant :
un mélange de fibres discontinues de polyester incluant une pluralité de premières fibres discontinues de polyester, une pluralité de deuxièmes fibres discontinues de polyester, et une pluralité de troisièmes fibres discontinues de polyester ;
dans lequel un denier de chacune des deuxièmes fibres discontinues de polyester est plus grand qu'un denier de chacune des premières fibres discontinues de polyester ;
dans lequel un denier de chacune des troisièmes fibres discontinues de polyester est plus grand qu'un denier de chacune des deuxièmes fibres discontinues de polyester ;
dans lequel chacune des premières fibres discontinues de polyester a un denier pas plus grand qu'environ 1 denier, chacune des deuxièmes fibres discontinues de polyester a un denier dans la plage de pas moins d'environ 1 denier à pas plus grand qu'environ 2 deniers, et chacune des troisièmes fibres discontinues de polyester a un denier de pas moins d'environ 2 deniers ;
dans lequel une longueur de sensiblement toutes les fibres discontinues de polyester du mélange est dans la plage d'environ 16 à environ 63 mm ;
dans lequel les fibres d'au moins l'une parmi les premières et deuxièmes fibres discontinues de polyester sont du téréphtalate de polyéthylène ;
dans lequel au moins une majorité des fibres discontinues de polyester du mélange sont ouvertes ; et
dans lequel les fibres comprenant le mélange sont séparées, individualisées et non liées les unes par rapport aux autres.

2. Matériau d'isolation soufflable selon la revendication 1, dans lequel le mélange comprend environ 20 à environ 40 pour cent en poids des premières fibres discontinues de polyester, environ 20 à environ 30 pour cent en poids des deuxièmes fibres discontinues de polyester, et environ 40 à environ 60 pour cent en poids des troisièmes fibres discontinues de polyester.

3. Matériau d'isolation soufflable selon la revendication 1, dans lequel la longueur de chacune des fibres discontinues de polyester du mélange est dans la plage d'environ 20 à environ 30 mm.

4. Matériau d'isolation soufflable selon la revendication 1, dans lequel au moins environ 95 % des fibres discontinues de polyester du mélange sont ouvertes.

5. Matériau d'isolation soufflable selon la revendication 1, dans lequel les fibres d'au moins l'une parmi les premières fibres discontinues de polyester et les deuxièmes fibres discontinues de polyester inclut un lubrifiant.

6. Matériau d'isolation soufflable selon la revendication 5, dans lequel le lubrifiant 5 est du silicone.

7. Matériau d'isolation soufflable selon la revendication 1, dans lequel les fibres d'au moins l'une parmi les premières fibres discontinues de polyester et les deuxièmes fibres discontinues de polyester sont frisées.

8. Matériau d'isolation soufflable selon la revendication 1, dans lequel le mélange présente une résistance au transfert de chaleur de duvet de force de rembourrage 700.

9. Article comprenant une enveloppe externe contenant un volume du matériau d'isolation soufflable selon la revendication 1.

10. Approvisionnement en matériau d'isolation pour le rembourrage d'au moins un segment d'une enveloppe d'un vêtement par le biais d'un appareil de soufflage, le matériau d'isolation comprenant :
un mélange de fibres discontinues de polyester incluant une pluralité de premières fibres discontinues de polyester, une pluralité de deuxièmes fibres discontinues de polyester, et une pluralité de troisièmes fibres discontinues de polyester ;
dans lequel un denier de chacune des deuxièmes fibres discontinues de polyester est plus grand qu'un denier de chacune des premières fibres discontinues de polyester ;
dans lequel un denier de chacune des troisièmes fibres discontinues de polyester est plus grand qu'un denier de chacune des deuxièmes fibres discontinues de polyester ;
dans lequel chacune des premières fibres discontinues de polyester a un denier pas plus grand qu'environ 1 denier, chacune des deuxièmes fibres discontinues de polyester a un denier dans la plage de pas moins d'environ 1 denier à pas plus grand qu'environ 2 deniers, et chacune des troisièmes fibres discontinues de polyester a un denier de pas moins d'environ 2 deniers ;
dans lequel une longueur de chacune des fibres discontinues de polyester du mélange est dans la plage d'environ 16 à environ 63 mm ;
dans lequel au moins une majorité des fibres discontinues de polyester du mélange sont ouvertes ; et dans lequel les fibres comprenant le mélange sont séparées, individualisées et non liées les unes par rapport aux autres.

11. Procédé de préparation d'un approvisionnement en matériau d'isolation soufflable, le procédé comprenant :
l'obtention d'une quantité de premières fibres discontinues de polyester ;
l'obtention d'une quantité de deuxièmes fibres discontinues de polyester ;
l'obtention d'une quantité de troisièmes fibres discontinues de polyester, dans lequel un denier moyen de chacune des deuxièmes fibres discontinues de polyester est plus grand qu'un denier moyen de chacune des premières fibres discontinues de polyester, dans lequel un denier moyen de chacune des troisièmes fibres discontinues de polyester est plus grand qu'un denier moyen de chacune des deuxièmes fibres discontinues de polyester,
dans lequel chacune des premières fibres discontinues de polyester a un denier pas plus grand qu'environ 1 denier, chacune des deuxièmes fibres discontinues de polyester a un denier dans la plage de pas moins d'environ 1 denier à pas plus grand qu'environ 2 deniers, et chacune des troisièmes fibres discontinues de polyester a un denier de pas moins d'environ 2 deniers, dans lequel chacune des premières fibres discontinues de polyester et chacune des deuxièmes fibres discontinues de polyester a une longueur dans la plage d'environ 16 à environ 63 mm, et dans lequel les fibres comprenant le mélange sont séparées, individualisées et non liées les unes par rapport aux autres ; et
le mixage des quantités de premières, deuxièmes, et troisièmes fibres discontinues de polyester pour fournir un mélange de fibres discontinues de polyester utiles en tant qu'un approvisionnement en matériau d'isolation soufflable.
